

# United States Patent Office

2,809,918

Patented Oct. 15, 1957

1

2,809,918

## SUSTAINED RELEASE PHARMACEUTICAL PREPARATIONS

Victor M. Hermelin, University City, Mo.

No Drawing. Application October 17, 1955,  
Serial No. 541,032

11 Claims. (Cl. 167—82)

This invention relates in general to certain new and useful improvements in pharmaceutical preparations and, more particularly, to a unique type of enteric coated beadlet containing a drug or medicament.

The medical profession frequently has need for drugs or medicaments which can be administered to the patient for purposes of achieving a very quick pharmacological therapeutic effect and will also maintain such effect over a prolonged period of time. Unfortunately, many drugs and particularly sedatives and hypnotics usually produce a sedated or narcotized condition of relatively short duration and are administered in comparatively light doses in order to avoid toxic reactions or other side effects which would be harmful to the patient. Similarly, there are some syndromes which may call for administration of a drug which should enter the patient's system in small doses at spaced intervals.

It is the primary object of the present invention, therefore, to provide a type of pharmaceutical preparation which is capable of producing both a quick initial effect and repetitive effect at spaced intervals over any desired or predetermined period of time.

It is another object of the present invention to provide a pharmaceutical preparation having the combined effects of prompt initial action and prolonged repetitive effect, which preparation is simple to administer, is relatively economical in cost of manufacture, and provides the physician with a very flexible type of *materia medica* from which to prescribe.

With the above and other objects in view, my invention resides in the novel features of form, construction, arrangement, and combination of parts presently described and pointed out in the claims.

Broadly speaking, the present invention resides in the discovery that it is possible to form a beadlet having a more or less spherical inactive core around which successive layers of the drug or medicament are built up, such layers being separated by enteric envelope-layers formed of a mixture of shellac and stearic acid. The enteric coatings or enveloping layers will resist the action of the fluids in the stomach and intestines for a predetermined period of time. The outer envelope containing the initial dose is preferably coated or encased in the usual readily soluble sugar coating capable of being dissolved in the stomach juices.

The following procedure is illustrative of the present invention:

20 lbs. screened cane sugar in coating pan

20 oz. colored simple syrup added

Pan rotated until mixed thoroughly

1 scoop ( $\frac{1}{2}$  lb.) powdered sugar and talc added

Air blown into coating pan during rotation cycle of about one-half hour.

Repeated 9 times, amounts of syrup varying from 20 oz. to 32 oz. and amounts of powdered sugar and talc (10%) varying from  $\frac{1}{2}$  lb. to 1 lb. at each application, depending on conditions. Time intervals (drying)

2

varying from 25 minutes to 35 minutes. An extra half hour of drying time added at end of run to assure all beads being dry.

Screened through 10 on 20 and 40 mesh screens.

5 Yield:

$\frac{1}{2}$  lb. on 10 mesh (tailings, agglomerates)

28 lbs. on 20 mesh

11 $\frac{1}{2}$  lbs. on 40 mesh

1 lb. through 40 mesh (fines)

10

41 lbs.

It will, of course, be understood that the above quantities are merely illustrative of the method by which the inactive cores are formed. It also should be pointed out that for any particular batch one size of bead should be used and the other sizes, which are screened out, should be used for other purposes or for other batches.

Thereupon, a weighed quantity of slow-release granules

20 made in accordance with the procedure described in my copending application Serial No. 541,027, filed contemporaneously herewith, are crushed finely, but not pulverized. Then, a weighed quantity of the inactive beads or cores are placed in a coating pan and the pan set in motion. A quantity of the shellac (3 lb. cut U. S. P. grade) is then poured into the pan sufficient to thoroughly wet the surfaces of the beads and, thereupon, a quantity of the crushed granules is introduced slowly into the pan until the wet surfaces of the beadlets are dried up. Then, 25 more of the shellac is added and again crushed granules are introduced until a second substantially dry coating has been formed. This procedure is repeated until the desired amount of crushed granules have been applied to the cores to form a mass of discrete beadlets.

30 35 If desired, the beadlets can be trimmed up by applying a conventional outer coating of colored sugar glaze. The above-described procedure can be applied in compounding any of the drugs or medicaments mentioned in the above-identified copending application.

40 45 It should be understood that changes and modifications in the form, construction, arrangement, and combination of the several parts of the pharmaceutical preparation may be made and substituted for those herein shown and described without departing from the nature and principle of my invention.

Having thus described my invention, what I claim and desire to secure by Letters Patent is:

1. The process for making sustained period minute-incremental dosage pharmaceutical preparations which 50 comprises intimately mixing a powdered drug and an enteric water insoluble excipient to produce a pasty mass, drying the mass slowly without agitation in such a manner as to produce a rough granular material, breaking up the rough granular material by light crushing, 55 whereby to reduce it to granular particles, said mixing, drying and crushing operations constituting one cycle, and remixing the granular particles with an additional quantity of the excipient to produce a pasty mass, re-drying such pasty mass slowly and without agitation in 60 such a manner as to produce a granular material, again breaking up the rough granular material by light crushing, whereby to reduce it again to granular particles, said second mixing, drying and crushing operations constituting a second cycle, said process consisting of not 65 less than three nor more than fifteen mixing, crushing and drying cycles repeated in successive order whereby to produce a pharmaceutical material consisting of granules having slow but continuous and attenuated solubility in the gastro-intestinal tract, lightly crushing said 70 finished granules to form a granular powder, forming a plurality of inert seed-like cores, placing said cores in a coating pan; rotating the coating pan, introducing

thereinto a water insoluble excipient, dusting in said granular powder, and continuing the addition of water insoluble excipient and granular powder until the desired dosage has been incorporated in the batch.

2. The process for making sustained period minute-incremental dosage pharmaceutical preparations which comprises intimately mixing a powdered drug and shellac to produce a pasty mass, drying the mass slowly without agitation in such a manner as to produce a rough granular material, breaking up the rough granular material by light crushing, whereby to reduce it to granular particles, said mixing, drying and crushing operations constituting one cycle, and remixing the granular particles with an additional quantity of shellac to produce a pasty mass, redrying such pasty mass slowly and without agitation in such a manner as to produce a granular material, again breaking up the rough granular material by light crushing, whereby to reduce it again to granular particles, said second mixing, drying and crushing operations constituting a second cycle, said process consisting of not less than three nor more than fifteen mixing, crushing and drying cycles repeated in successive order whereby to produce a pharmaceutical material consisting of granules having slow but continuous and attenuated solubility in the gastro-intestinal tract, lightly crushing said finished granules to form a granular powder, forming a plurality of inert seed-like cores, placing said cores in a coating pan, rotating the coating pan, introducing thereinto shellac, dusting in said granular powder, and continuing the addition of shellac and granular powder until the desired dosage has been incorporated in the batch.

3. The process for making sustained period minute-incremental dosage pharmaceutical preparations which comprises intimately mixing a powdered drug and an enteric water insoluble excipient consisting of a mixture of shellac and stearic acid, whereby to produce a pasty mass, drying the mass slowly without agitation in such a manner as to produce a rough granular material, breaking up the rough granular material by light crushing, whereby to reduce it to granular particles, said mixing, drying and crushing operations constituting one cycle, and remixing the granular particles with an additional quantity of the excipient to produce a pasty mass, redrying such pasty mass slowly and without agitation in such a manner as to produce a granular material, again breaking up the rough granular material by light crushing, whereby to reduce it again to granular particles, said second mixing, drying and crushing operations constituting a second cycle, said process consisting of not less than three nor more than fifteen mixing, crushing and drying cycles repeated in successive order whereby to produce a pharmaceutical material consisting of granules having slow but continuous and attenuated solubility in the gastro-intestinal tract, lightly crushing said finished granules to form a granular powder, forming a plurality of inert seed-like cores, placing said cores in a coating pan, rotating the coating pan, introducing thereinto a water insoluble excipient, dusting in said granular powder, and continuing the addition of water insoluble excipient and granular powder until the desired dosage has been incorporated in the batch.

4. The process for making sustained period minute-incremental dosage pharmaceutical preparations which comprises intimately mixing a powdered drug and an enteric water insoluble excipient to produce a pasty mass, placing the mass on trays and drying the mass slowly without agitation in such a manner as to produce a rough granular material, breaking up the rough granular material by light crushing, whereby to reduce it to granular particles, said mixing, drying and crushing operations constituting one cycle, and remixing the granular particles with an additional quantity of the excipient to produce a pasty mass, redrying such pasty

mass slowly and without agitation in such a manner as to produce a granular material, again breaking up the rough granular material by light crushing, whereby to reduce it again to granular particles, said second mixing, drying and crushing operations constituting a second cycle, said process consisting of not less than three nor more than fifteen mixing, crushing and drying cycles repeated in successive order whereby to produce a pharmaceutical material consisting of granules having slow but continuous and attenuated solubility in the gastro-intestinal tract, lightly crushing said finished granules to form a granular powder, forming a plurality of inert seed-like cores, placing said cores in a coating pan, rotating the coating pan, introducing thereinto a water insoluble excipient, dusting in said granular powder, and continuing the addition of water insoluble excipient and granular powder until the desired dosage has been incorporated in the batch.

5. The process for making sustained period minute-incremental dosage pharmaceutical preparations which comprises intimately mixing a powdered drug and an enteric water insoluble excipient to produce a pasty mass, spreading the mass in a thin layer upon trays and drying the mass slowly without agitation in such a manner as to produce a rough granular material, breaking up the rough granular material by light crushing, whereby to reduce it to granular particles, said mixing, drying and crushing operations constituting one cycle, and remixing the granular particles with an additional quantity of the excipient to produce a pasty mass, redrying such pasty mass slowly and without agitation in such a manner as to produce a granular material, again breaking up the rough granular material by light crushing, whereby to reduce it again to granular particles, said second mixing, drying and crushing operations constituting a second cycle, said process consisting of not less than three nor more than fifteen mixing, crushing and drying cycles repeated in successive order whereby to produce a pharmaceutical material consisting of granules having slow but continuous and attenuated solubility in the gastro-intestinal tract, lightly crushing said finished granules to form a granular powder, forming a plurality of inert seed-like cores, placing said cores in a coating pan, rotating the coating pan, introducing thereinto a water insoluble excipient, dusting in said granular powder, and continuing the addition of water insoluble excipient and granular powder until the desired dosage has been incorporated in the batch.

6. The process for making sustained period minute-incremental dosage pharmaceutical preparations which comprises intimately mixing a powdered drug and an enteric water insoluble excipient to produce a pasty mass, spreading the mass in a thin layer upon air pervious trays and drying the mass slowly without agitation in such a manner as to produce a rough granular material, breaking up the rough granular material by light crushing, whereby to reduce it to granular particles, said mixing, drying and crushing operations constituting one cycle, and remixing the granular particles with an additional quantity of the excipient to produce a pasty mass, redrying such pasty mass slowly and without agitation in such a manner as to produce a granular material, again breaking up the rough granular material by light crushing, whereby to reduce it again to granular particles, said second mixing, drying and crushing operations constituting a second cycle, said process consisting of not less than three nor more than fifteen mixing, crushing and drying cycles repeated in successive order whereby to produce a pharmaceutical material consisting of granules having slow but continuous and attenuated solubility in the gastro-intestinal tract, lightly crushing said finished granules to form a granular powder, forming a plurality of inert seed-like cores, placing said cores in a coating pan, rotating the coating pan, introducing thereinto a water insoluble excipient, dusting in said

granular powder, and continuing the addition of water insoluble excipient and granular powder until the desired dosage has been incorporated in the batch.

7. The process for making sustained period minute-incremental dosage pharmaceutical preparations which comprises intimately mixing a powdered drug and an enteric water insoluble excipient to produce a pasty mass, spreading the mass in a thin layer upon cloth bottom trays and drying the mass slowly without agitation in such a manner as to produce a rough granular material, breaking up the rough granular material by light crushing, whereby to reduce it to granular particles, said mixing, drying and crushing operations constituting one cycle, and remixing the granular particles with an additional quantity of the excipient to produce a pasty mass, redrying such pasty mass slowly and without agitation in such a manner as to produce a granular material, again breaking up the rough granular material by light crushing, whereby to reduce it again to granular particles, said second mixing, drying and crushing operations constituting a second cycle, said process consisting of not less than three nor more than fifteen mixing, crushing and drying cycles repeated in successive order whereby to produce a pharmaceutical material consisting of granules having slow but continuous and attenuated solubility in the gastro-intestinal tract, lightly crushing said finished granules to form a granular powder, forming a plurality of inert seed-like cores, placing said cores in a coating pan, rotating the coating pan, introducing thereinto a water insoluble excipient, dusting in said granular powder, and continuing the addition of water insoluble excipient and granular powder until the desired dosage has been incorporated in the batch.

8. The process for making sustained period minute-incremental dosage pharmaceutical preparations which comprises intimately mixing a powdered drug and an enteric water insoluble excipient to produce a pasty mass, drying the mass slowly without agitation in a hot dry atmosphere in such a manner as to produce a rough granular material, breaking up the rough granular ma-

terial by light crushing, whereby to reduce it to granular particles, said mixing, drying and crushing operations constituting one cycle, and remixing the granular particles with an additional quantity of the excipient to produce a pasty mass, redrying such pasty mass slowly and without agitation in such a manner as to produce a granular material, again breaking up the rough granular material by light crushing, whereby to reduce it again to granular particles, said second mixing, drying and crushing operations constituting a second cycle, said process consisting of not less than three nor more than fifteen mixing, crushing and drying cycles repeated in successive order, whereby to produce a pharmaceutical material consisting of granules having slow but continuous and attenuated solubility in the gastro-intestinal tract, lightly crushing said finished granules to form a granular powder, forming a plurality of inert seed-like cores, placing said cores in a coating pan, rotating the coating pan, introducing thereinto a water insoluble excipient, dusting in said granular powder, and continuing the addition of water insoluble excipient and granular powder until the desired dosage has been incorporated in the batch.

9. A pharmaceutical preparation made in accordance with the process of claim 1.

10. A pharmaceutical preparation made in accordance with the process of claim 2.

11. A pharmaceutical preparation made in accordance with the process of claim 3.

#### References Cited in the file of this patent

#### UNITED STATES PATENTS

|           |               |               |
|-----------|---------------|---------------|
| 312,041   | Upjohn        | Feb. 10, 1885 |
| 1,012,788 | Zwingenberger | Dec. 26, 1911 |
| 2,052,376 | Zellers       | Aug. 25, 1936 |
| 2,736,682 | Hermelin      | Feb. 28, 1956 |

#### OTHER REFERENCES

- Little et al.: Tablet Making (Liverpool, 1949), pp. 42 and 43.  
 Clarkson: Tablet Coating (New York, 1951), p. 61.